

# UNITED STATES PATENT OFFICE.

ANTOINE LAVOCAT, OF LYONS, FRANCE.

## COMPOSITION FOR CLOSING PUNCTURES IN PNEUMATIC TIRES.

SPECIFICATION forming part of Letters Patent No. 618,694, dated January 31, 1899.

Application filed September 28, 1898. Serial No. 692,115. (No specimens.)

*To all whom it may concern:*

Be it known that I, ANTOINE LAVOCAT, chemist, a citizen of the Republic of France, residing in Lyons, (Rhône,) France, have invented a new and Improved Puncture-Closing Composition for Use in Connection with Pneumatic Tires and the Like, which is fully set forth in the following specification.

This invention relates to a composition intended for stopping leaks in the air-chambers of tires for velocipedes or in india-rubber tubes or pipes subject to rupture.

My improved composition, which I term "Steganol," is intended to be introduced into the air-chambers of pneumatic tires for the purpose of stopping automatically, instantaneously, and hermetically holes or punctures accidentally made.

The composition is as follows: gutta percha, one thousand grams; copaiba or other balsam, four thousand grams; holly or other bird-lime,

four thousand grams; Swiss or Bordeaux turpentine, two thousand grams; saturated solution of celluloid, four thousand grams; chloroform or any other solvent, a quantity sufficient to dissolve the gutta-percha and other substances above mentioned.

I prefer chloroform to any other solvent.

I claim—

The herein-described composition of matter, consisting of gutta-percha, a balsam, bird-lime, turpentine, a saturated solution of celluloid, and a suitable solvent, in substantially the proportions specified.

In testimony whereof I have signed this specification in the presence of two subscribing witnesses.

ANTOINE LAVOCAT.

Witnesses:

LOUIS MAYNARD,  
JEAN BAIRO.